

# UNITED STATES PATENT OFFICE.

ANDREW DERROM, OF PATERSON, NEW JERSEY.

COMPOSITION MASTIC FOR COVERING ROOFS, TELEGRAPH-WIRES, AND THE LIKE.

SPECIFICATION forming part of Letters Patent No. 307,184, dated October 28, 1884.

Application filed April 15, 1884. (Specimens.)

*To all whom it may concern:*

Be it known that I, ANDREW DERROM, a resident of Paterson, in the county of Passaic and State of New Jersey, have invented an 5 Improved Composition Mastic for Covering Roofs, Telegraph-Wires, and the like, of which the following is a full, clear, and exact specification.

This invention relates to a new mixture of 10 two peculiar natural products which are found along the northern part of South America. These are, first, a hard Venezuelan bituminous deposit, known as "crude hard Venezuelan bitumen," found in Venezuela and on the north 15 coast of South America, or other hard crude asphaltum; secondly, soft bitumen that flows by volcanic action in a lake near Maturin, Venezuela. The soft bitumen is first refined and then boiled, and the hard bitumen is then 20 melted in the boiled soft bitumen. The best proportions are about ten parts of soft to five parts, by measure, of the hard bitumen; but good results have also been obtained by mix-

ing ten parts of the soft, with two parts of the hard, and two parts of the soft, with ten parts 25 of the hard, bitumen. The mixture is peculiarly adhesive and very elastic and pliable, and furnishes an excellent ductile covering for telegraph-wires, roofs, and the like. The soft bitumen alone is not useful, because it cannot 30 be made hard or plastic except at very great expense. The hard bitumen alone cannot be used as a pliable ingredient unless mixed with oils, which are more liable to disintegrate than is the soft bitumen. The mixture of the two 35 kinds of bitumen mentioned by me is wholly free from smell, and therefore particularly advantageous.

I claim—

The composition of hard bituminous deposit 40 and purified soft Venezuelan bitumen in the proportions specified.

ANDREW DERROM.

Witnesses:

WILLY G. E. SCHULTZ,  
HARRY M. TURK.